

Aug. 11, 1931.

H. H. STOUT

1,817,935

PYROMETALLURGICAL COPPER REFINING

Filed Aug. 15, 1928

2 Sheets-Sheet 1



Aug. 11, 1931.

H. H. STOUT

1,817,935

PYROMETALLURGICAL COPPER REFINING

Filed Aug. 15, 1928

2 Sheets-Sheet 2



## UNITED STATES PATENT OFFICE

HARRY H. STOUT, OF CLIFTON, ARIZONA, ASSIGNOR TO COPPER DEOXIDATION CORPORATION, OF NEW YORK, N. Y., A CORPORATION OF NEW YORK

## PYROMETALLURGICAL COPPER REFINING

Application filed August 15, 1928. Serial No. 299,666.

This invention relates to the pyrometallurgical refining of copper.

This application is in part a continuation of my prior applications Ser. No. 607,427, filed Dec. 16, 1922, and Ser. No. 111,887, filed May 26, 1926.

The object of the invention is to produce at less cost a fire-refined product with chemical and physical properties superior to those of the product of previously known refining methods.

A particular object is to produce a copper having uniform and dependable physical qualities, a result which cannot be reached by prior art fire-refining practice.

In the drawings:

Figure 1 is a diagram representing the location of the different units used in carrying out the invention.

Figure 2 is an elevation partly in section of certain pieces of apparatus.

Figure 3 is a section of a line 3—3 of Figure 2.

During the oxidizing, poling, and casting periods in the reverberatory furnaces used for present fire refining practice, fuel gases are in contact with the molten metal. Since it is impossible to obtain fuel and burn it in such manner that its gases do not contain partial pressures of the detrimental substances such as sulphur, oxygen, sulphur dioxide, carbon dioxide, hydrogen sulphide, water vapor and hydrocarbons, it follows that it is impossible to produce a product free from them.

The absorption of these impurities by contact with the fuel gases is reduced by using large capacity casting machines and thus shortening the exposure time, but this remedy has physical limitations.

By lowering the temperature, the absorption of impurities is reduced, but if the temperature of the copper is lowered in the furnace below about 1170° C., the metal freezes on the ladle lips in pouring.

Another source of contamination of present process fire refined copper is the oxygen absorbed by the molten metal in transit from the interior of the furnace to the mould and

during the solidification in the mould. My experimentation on this point disclosed:

A. Previous investigators and present practice operators believe the amount of oxygen absorbed by the molten copper in transit from the furnace and in the mould is negligible. This conclusion was arrived at by comparing "poured sample" with "product sample". The "poured sample" itself often absorbs more oxygen than the product due to its diminished "pouring rate".

B. I have proved by accurate technique in obtaining a true sample of the copper in the furnace, that the amount of oxygen thus absorbed is very appreciable. Depending on the "pouring rate" and on the "cascade rate", I have found it to vary in the refined copper product (not considering anodes) of present practice fire refining plants approximately as follows: expressed in per cent. of metal product,

|                           |                |
|---------------------------|----------------|
| O content in furnace from |                |
| about                     | 0.032 to 0.022 |
| O absorbed from air       | 0.008 .018     |

O content product 0.040 0.040

C. Not all of the oxygen thus absorbed is converted into O<sub>2</sub> because the time before solidification is not sufficient; hence part of it remains as Cu<sub>2</sub>O flakes or crystals.

My experimentation disclosed that in the present fire refining practice a readjustment in the elements and compounds in the molten copper occurs during its transit from the furnace and during the solidification in the mould, as follows:

A. Reduction of H partial pressure from fuel gases to atmosphere and cooling of the metal causes liberation of H upon emerging from the furnace which continues until solidification occurs. If solidification is too rapid, H is entrapped producing gas pockets.

B. Increased O partial pressure in atmosphere over that in the fuel gases, causes O absorption as explained above and equilibrium readjustment begins.

C. As the temperature of the metal from the furnace and in the mould falls, the various substances present crystallize out at or

below their melt points as illustrated by the following:

|                                  |          |
|----------------------------------|----------|
| First.—Excess Cu <sub>2</sub> O  | 1210° C. |
| Second.—Excess Cu <sub>2</sub> S | 1127° C. |
| Third.—Excess copper crystals    | 1083° C. |
| Fourth.—S.Eu                     | 1067° C. |
| Fifth.—O.Eu                      | 1064° C. |

(S.Eu=copper-cuprous sulphide eutectic)  
(O.Eu=copper-cuprous oxide eutectic)

- 10 D. As each one of the substances is withdrawn, by crystallization, readjustment of equilibrium begins. When the excess copper crystallizes at about 1083° C., it leaves the 15 two eutectics (sulphide and oxide) as liquids separating the copper crystals. During the fall in temperature from about 1083° C. to 1067° C., the two liquid eutectics react upon each other to readjust the equilibrium as follows:



- Solidification of these eutectics at 1067° C. and 1064° C. puts an end to the readjustment. 25 Part of the SO<sub>2</sub> thus liberated escapes but part is entrapped and appears as gas pockets in the matrix areas between the dendrites.

- 30 My experimentation disclosed that for the same sulphur content in molten copper in the reverberatory furnaces used in present fire refining practice, the relative amounts of O.Eu present influences the per cent. of the total sulphur which enters into S.Eu solution and the per cent. which remains as Cu<sub>2</sub>S. 35 A. Raising the oxygen content of the molten copper in the furnace diminishes the per cent. of the total sulphur content which enters into S.Eu solution; hence less SO<sub>2</sub> gas is generated during solidification and the 40 surface of the bar is flat or concave—"low pitch copper."

- B. Lowering the oxygen content has the opposite effect and the surface of the bar is slightly convex—"high pitch copper."

- 45 C. An exaggerated form of B is known as "overpoled" or "sulphur worm" copper and this condition of excess S.Eu solution having occurred in the molten copper in the presence of the partial S pressure of the fuel gases, it 50 is necessary to completely reoxidize the charge in order to unbalance the S.Eu solution equilibrium and then again pole the metal.

- 55 My experimentation as outlined above discloses the fact and the reasons why it is physically impossible to produce by present practice fire refining methods a cast copper product which does not contain certain very detrimental impurities. It follows that the refiner makes a compromise product which the fabricator will accept because he can obtain no better, but which possesses physical characteristics which result in high fabricating 60 costs and excessive rejects.

The average American present practice fire refined product is about as follows:

A. Contains approximately 6.4% by volume of gas pockets.

B. Cuprous oxide flakes, not in eutectic solution, appear sparingly throughout the mass, with no particular crystalline arrangement.

C. Occasional strings of cuprous sulphide are similarly present.

D. Copper crystals comprise about 90% of the weight.

E. The matrix of O.Eu constitutes about 9% of the weight.

F. Some S.Eu is found at dendrite boundaries.

G. It is not homogeneous, the relative amounts of Cu<sub>2</sub>O, Cu<sub>2</sub>S, O.Eu, S.Eu and gas pockets vary widely in different parts of the same bar; hence rejection of ductility tests by A. S. T. M.

Summarizing the disclosure of my experimentation on the causes of physical imperfections of present practice fire refined product, these defects are caused by the presence in the product of Cu<sub>2</sub>O, O.Eu, Cu<sub>2</sub>S, S.Eu, H. These substances are formed from the presence in the copper of the following elements,—sulphur, oxygen, hydrogen.

If these three elements can be substantially removed from the copper at suitable points in the operation and thereafter, until solidification, the metal be not subjected to a partial pressure of these elements, which will cause reabsorption, a product free from the physical defects caused by these elements and/or their compounds can be produced. This result can be attained by the process disclosed hereinafter.

In carrying out the process, molten copper melted by any of the methods now used in the art and/or molten copper from the converter 10 is transported by the ladle 11 and poured through the launder 12 into the oxidizing vessel 13, which has been preheated by any suitable method. The preheating has been carried to such a point that the combined heat of the vessel and that of the entering copper results in a copper temperature of from about 2000° to 2050° F.

The copper is then oxidized by any of the methods now used in the art, such as by air and/or oxygen to about a saturated liquid solution of copper cuprous oxide eutectic at the particular temperature, thereby removing substantially all of the sulphur with the least addition of oxygen. The degree of oxidation necessary to remove substantially all sulphur is a function of the temperature of the copper at the finish of the blow, the lower the copper temperature, the lower the oxygen content necessary; in practice we have about 0.55% oxygen at 2030° F. The particular temperature used at the end of the oxidation is that found most economical un-

der the local conditions of fuel cost, wages, necessary tonnage per vessel, which is claimed per se in my copending application Serial No. 547,013, filed June 26, 1931, for 5 Vessel for fire refining, etc.

The oxidizing vessel is specially heat-insulated (as hereinafter disclosed) to prevent rapid loss of heat from the copper, and in some cases it is preferred to pour the oxidized copper without further heating into the reducing vessel 14. But the copper cuprous oxide eutectic may be heated by the combustion of commercial fuel to any desired temperature before it is transferred to 15 the subsequent vessel, if found desirable, as the copper will not absorb appreciable amounts of sulphur from the combustion gases while in the eutectic condition.

The oxidized copper is then transferred to 20 the reducing vessel 14 through the launder

15. This flow is caused by tilting the oxidizing vessel by means of hydraulic cylinder

16. The reducing vessel has been pre-heated to such a degree that the heat of the vessel 25 plus the heat of the incoming charge produces a copper temperature of about 2230 to 2275° F., a temperature high enough that after reduction and until casting is complete no application of heat to the copper is necessary.

After the eutectic is in the reducing vessel and before reduction begins it may be fired on by flame from commercial fuel as the eutectic as such will not absorb appreciable 30 amounts of sulphur beyond that which is substantially expelled by the hydrogen content of the reduction medium during the early stages of reduction when the oxygen content of the copper is relatively high.

40 When heating the empty reducing vessel and/or in heating the eutectic in the reducing vessel by application of commercial fuel flame, it was found that fuel of relatively high sulphur content can be used if the combustion gases have a suitable excess oxygen content.

In this vessel the eutectic is reduced to any desired oxygen content by any of the means now used in the art such as poles, charcoal, 45 suitable reducing gases, etc., and from this vessel the refined copper is cast by any of the means now used in the art which will cast the charge in a suitably short casting period time. For example, the vessel 14 may be moved 50 along track 17 and the copper poured into molds 18.

The oxidation and reduction can be performed in the same vessel, and the copper cast without subjecting it to contact with 55 flame from combustion of commercial fuel after reduction provided the vessel is suitably heat insulated and the casting period sufficiently short, but in this case the interior brick lining of the vessel will absorb appreciable sulphur from the copper before it is

oxidized and this sulphur will reenter the copper from the brick work during the latter stages of reduction, and the product contains relatively more sulphur than the product when oxidation and reduction are conducted 70 in separate vessels. On the other hand the product, even when oxidation and reduction are performed in the same vessel, contains appreciably less sulphur and is of superior 75 quality to the product of prior art practice due to its not being contaminated, during and after reduction, by contact with the combustion gases of commercial fuel. When oxidation is done in the first vessel there is no appreciable sulphur in the copper cuprous oxide eutectic when it enters the reducing vessel and hence the brick work of the reducing vessel is not contaminated with sulphur, and the resulting product is substantially 80 sulphur free.

It was found that if after reduction is completed to any desired point no flame is allowed to come in contact with the copper, the hydrogen in solution, from the reducing medium used, escapes from the copper, without the necessity of degasification, and does not appear as blow holes in the product. If, on the other hand, the flame is in contact with the copper during casting, such hydrogen will not escape from the copper and will appear 95 as blow holes in the product.

It was found that in order to maintain the molten copper in the reducing vessel after reduction and during casting at the required 100 temperature for proper casting operations, the vessel must be especially insulated against loss of heat and must have its openings necessary to conduct the process, capable of being closed relatively tight against the entrance of air into the vessel during the casting period; otherwise fuel is necessary during the casting period, which, as has been pointed out, poisons the copper when in the reduced condition.

It was found that any heat insulating material used in the construction of the vessels became impregnated with copper due to the molten copper penetrating between the joints in the brick work and as soon as this occurred the heat insulating qualities were 115 materially affected. One remedy for this was to increase the thickness of the brick lining to the point where the penetrating molten copper solidified before reaching the heat insulating material; the thickness of brick which this method required was so great that the vessel became so large as to become economically unworkable.

A practicable solution was reached by constructing the vessels in the following manner:

The inner lining 19, which is in contact with the molten copper is formed of basic brick; next comes a lining 20 of refractory brick and then a shell 21 preferably formed of chromium steel, or other resistant metal.

The lining 20 of refractory brick is of such a thickness that the steel shell 21 never rises above a temperature that it is well able to withstand over long periods of use. The 5 steel shell extends a safe distance above the molten copper level. The next lining 22 of the vessel is composed of a suitable heat-insulating material such as sil-o-cel, magnesium, asbestos, etc., and this lining must be 10 of suitable thickness to retain most of the heat within the vessel and at the same time permit the steel shell 21 to stay below its suitable working temperature. Outside of 15 this heat-insulating material is the outer metal shell 23. The oxidizing and reducing vessels may both be constructed in this manner.

This construction prevents the penetration 20 of the heat insulating material by the copper and the fuel economy resulting is shown by 25 the fact that prior art furnaces receiving molten blister from a converter and fire refining it in the prior art furnaces requires from 95 to 120 pounds of fuel oil per ton of 25 refined cast product in the process, while the vessel disclosed uses from 15 to 19 pounds of fuel oil per ton of refined cast product.

The present process differs from prior art 30 practice also in that prior art requires a much higher capital expenditure per ton of product as the following example will show. To produce 240 tons per day of product, fire refined from molten blister, requires by prior art 35 methods two furnaces of 120 tons each or 240 tons total, from each furnace one charge in 24 hours is cast and the casting period is from 3 to 5 hours long for each charge. With my process two vessels each approximately 20 tons or a total vessel size of 40 tons, will cast 40 the same amount of copper, a charge is cast every two hours and the casting period for each charge is from 18 to 26 minutes.

The large size furnace units of the prior art 45 require continuous combustion of fuel and therefore need an oxidizing flame during reduction and casting. They consume from 52 to 83 pounds of poles per ton of product. In the present process no fuel is required during reduction and casting, only from 23 to 32 pounds of poles are used per ton of product, and the length of time required for reduction 55 is correspondingly shorter.

In order to produce deoxidized billets, cake, etc., by the use of soluble deoxidizers, prior 60 art practice necessitates the hand ladling and hand casting of such deoxidized copper and the addition of the soluble deoxidizer in the hand ladle and/or in the hand poured crucible. This is because the combustion contact 65 of oxidizing combustion gases of commercial fuel during the casting period in prior art furnaces oxidizes the soluble deoxidizer as rapidly as it is added to the molten copper. In the present process any of the soluble de- 75 oxidizers now used in the art, such as phos-

phorus, silicon, zinc, etc., can be added to the 70 previously substantially deoxidized copper in the furnace and the copper cast in the same manner as any other form of copper, thus eliminating the very expensive hand ladling and hand casting of deoxidized copper.

The excess amount of such soluble deoxidizers in the deoxidized copper in the furnace is only that which by the casting methods used 75 will fix as an oxide of the soluble deoxidizer all oxygen absorbed by the molten copper in transit from the furnace into the mould and during solidification in the mould.

I claim:

1. The process of fire refining copper which 80 includes chemically reducing previously oxidized molten copper without applying heat to the copper after the start of the reducing step.

2. The process of fire refining copper which 85 includes chemically reducing previously oxidized molten copper in a vessel having a basic inner lining without applying heat to the copper after the start of the reducing step.

3. The process of fire refining copper which 90 includes chemically reducing previously oxidized molten copper in a vessel having a basic inner lining and a heat-insulating outer layer without applying heat to the copper after 95 the start of the reducing step.

4. The process of fire refining copper which 100 includes chemically reducing previously oxidized molten copper without applying heat to the copper after the oxygen content is reduced below 0.2%.

5. The process of fire refining copper which 105 includes chemically reducing previously oxidized molten copper and casting the copper without applying heat to the copper after the start of the reducing step.

6. The process of fire refining copper which 110 includes pouring previously melted molten copper containing sulphur into a vessel and oxidizing it to a saturated solution of copper cuprous oxide eutectic, at a temperature below 2075° F. and above 2000° F., thereafter heating the copper to a temperature in excess of 2150° F. by burning commercial fuel inside the vessel, transferring the molten copper to a second vessel, and chemically reducing the copper in the second vessel.

7. The process of fire refining copper which 115 includes pouring previously melted molten copper containing sulphur into a vessel having an inner refractory basic lining and an outer heat-insulating lining and oxidizing it to a saturated solution of copper cuprous oxide eutectic, at a temperature below 2075° F. and above 2000° F., thereafter heating the copper to a temperature in excess of 2150° F. by 120 burning commercial fuel inside the vessel, transferring the molten copper to a second vessel having an inner refractory basic lining and an outer heat-insulating lining and 125

130

chemically reducing the copper in the second vessel.

8. The process of fire refining copper which includes pouring previously melted molten copper containing sulphur into a vessel and oxidizing it to a saturated solution of copper cuprous oxide eutectic, at a temperature below 2075° F. and above 2000° F., transferring the molten copper to a second vessel, and
- 10 chemically reducing the copper in the second vessel, sufficient additional heat having been supplied to the copper after the oxidizing step to avoid the necessity of adding additional heat during the reducing step.
- 15 9. The process of fire refining copper which consists of oxidizing molten copper to approximately a saturated liquid solution of copper cuprous oxide eutectic at approximately 2030° F., transferring the copper to a
- 20 heat-insulated vessel, chemically reducing the copper and casting it, sufficient additional heat having been supplied to the copper after the oxidizing step and before the start of the reducing step to avoid the necessity of adding additional heat during the reducing step.
- 25

In testimony whereof I affix my signature.  
**HARRY H. STOUT.**

30

35

40

45

50

55

60

65